

R. GAHL.

PROCESS OF CONCENTRATING OXID ORES OF COPPER.

APPLICATION FILED DEC. 27, 1916.

1,217,437.

Patented Feb. 27, 1917.



Witness

G. J. Baker

Rudolf Gahl

By Bruce Townsend & Dickstein

Attorneys

# UNITED STATES PATENT OFFICE.

RUDOLF GAHL, OF MIAMI, ARIZONA.

## PROCESS OF CONCENTRATING OXID ORES OF COPPER.

1,217,437.

Specification of Letters Patent. Patented Feb. 27, 1917.

Application filed December 27, 1916. Serial No. 139,148.

*To all whom it may concern:*

Be it known that I, RUDOLF GAHL, a citizen of the United States, residing at Miami, in the county of Gila and State of Arizona, 5 have invented certain new and useful Improvements in Processes of Concentrating Oxid Ores of Copper, of which the following is a specification.

My invention relates to a process for 10 treating copper ores of the oxid type to make them amenable to flotation. These so-called oxid ores (cuprite, tenorite, malachite, azurite, etc.) in contradistinction to the sulfid ores are not ordinarily capable of 15 concentration by flotation.

The process consists in agitating the ground ore or pulp to which flotation oil 20 may have already been added, in the presence of an acid, such as sulfuric acid, which dissolves the soluble copper constituents of 25 the ore. The agitation may be readily effected by blowing air into the vessel containing the ore pulp. The pulp is then subjected to the action of finely divided iron, obtained in any suitable manner, as in the 30 form of filings, or the fine iron resulting from the action of steel balls in ball mills, or sponge iron formed by the reduction of iron oxids by carbon or oil at a temperature below the melting point of iron.

The result of the addition of the iron to 35 the pulp is to cause the precipitation of cement copper from the acid solution. The iron is then separated from the pulp in any suitable manner, as by a magnetic separator. The pulp from which the iron has been separated is then treated in a flotation machine which may be of any of the well-known constructions.

40 The cement copper and copper-sulfids, if any, present in the pulp are separated by the flotation operation and collected in the usual way.

This treatment may be combined with 45 any of the known processes of ore concentration, for instance, the pulp may undergo a preliminary table or other gravity treatment, or a preliminary flotation before the acid treatment above described. The tailings produced may be subjected to either gravity or flotation concentration.

Any suitable apparatus may be employed, 50 one form designed for continuous operation being shown in the accompanying drawings in which A is an agitating tank, which may be divided by partitions 2, into several com-

partments, into each of which air under pressure is introduced through pipes 3 connected to an air-main 4.

The ore-pulp and acid are introduced at 60 the head-end of the tank through pipes 5 and 6. The pulp travels in succession through the compartments and is delivered through pipe 7 to a precipitating tank B similar in construction to the agitating tank 65 A and also provided with agitating means. From the precipitating tank B, the pulp is delivered by pipe 8 and launder 9 to the magnetic separator C, by which the iron which has not been dissolved is removed. 70 Any suitable form of magnetic separator may be used, such as a belt 10 traveling over a magnetized pulley 11. The iron which is separated is delivered by hopper 12 into a receptacle 13, from which it may be conducted by any suitable elevator 14 to the head end of the tank B, for re-use. The unmagnetic portion of the pulp, passes over plate 15 to a flotation machine D, which may be of any of the well known constructions, 75 such as the beater or pneumatic types. The function of the magnetic separator is not only to economize in iron consumption, but mainly to keep up an appreciable return of iron to the tank B, for the purpose of 80 maintaining in the same, a high percentage of iron particles, although the quantity of iron added in the form of fresh iron may be small. A large surface of metallic iron will thus be constantly exposed to the copper solutions in the precipitating tank B, and the reaction will, accordingly take place 85 rapidly. In this manner an agitating tank of very small dimensions serves the purpose of precipitating the copper contained in a 90 large amount of pulp. The flotation machine D produces a concentrate consisting mainly of cement copper, in case there are 95 being treated ores, such as what are known as oxid ores, the copper contents of which 100 are essentially soluble in sulfuric acid. If, however, sulfids are present in the ore, they will go into the concentrate along with the cement copper.

I claim:—

1. The process of concentrating oxid ores of copper which consists in adding thereto acid to dissolve the soluble copper ingredients, precipitating the copper from solution by iron, separating the undissolved 110 iron from the pulp, and subjecting the residue to a flotation operation.

105

2. The process of concentrating oxid ores of copper which consists in adding thereto acid to dissolve the soluble copper ingredients, precipitating the copper from solution by iron, magnetically separating the undissolved iron from the pulp, and subjecting the residue to a flotation operation.
3. The process of concentrating oxid ores of copper which consists in adding thereto acid to dissolve the soluble copper ingredients, precipitating the copper from solution by iron, separating the undissolved iron from the pulp, re-using the recovered iron for further precipitation, and subjecting the residue to a flotation operation.
4. The continuous process of concentrating oxid ores of copper which consists in agitating the pulp in the presence of acid, precipitating the copper from the pulp by metallic iron, magnetically separating the undissolved iron, re-using the thus recovered metallic iron for further precipitation, and subjecting the pulp containing the cement-copper to flotation.

In testimony whereof I affix my signature in presence of two witnesses.

RUDOLF GAHE.

Witnesses:

F. S. TRELOAR,  
A. REID.